

## UNITED STATES PATENT OFFICE

2,152,460

## MANUFACTURE OF PHOTOGRAPHIC GELATIN EMULSIONS

Emil Joachim Birk, Bitterfeld, and Hans Fricke and Gustav Wilmanns, Wolfen, Kreis Bitterfeld, Germany, assignors to Agfa Ansco Corporation, Binghamton, N. Y., a corporation of New York

No Drawing. Application July 10, 1935, Serial No. 30,636. In Germany July 14, 1934

3 Claims. (Cl. 95—7)

Our present invention relates to the manufacture of photographic gelatin emulsions.

One of its objects is to provide an improved photographic gelatin emulsion free from fog. Further objects will be seen from the detailed specification following hereafter.

It is known that some kinds of gelatin are not useful for the production of photographic emulsions owing to the fact that in the course of the usual process for producing the emulsion the emulsion suffers an extensive fogging, which is apparently due to the presence in the natural gelatin of too high a proportion of substances which promote ripening.

According to this invention a gelatin of this kind can be rendered suitable for use for the production of photographic emulsions with good results, by adding to the gelatin or to the emulsion at any desired stage in the preparation of the gelatin or emulsion, an amino-purine such as guanine or adenine, or mixtures of these compounds. By the addition of one of these substances the tendency towards fogging is so strongly diminished that gelatin of this kind can be worked up into emulsions of all kinds in the same manner as a photographic gelatin of the highest grade. The compounds are added in the form of solutions. Suitable solvents are water and alcohols and may be made alkaline by the addition of a small quantity of caustic soda.

The proportion of the substance to be added is adjusted according to the extent to which the gelatin or emulsion undergoes fogging, previously determined in the usual manner.

The following examples illustrate the invention:

Example 1.—To a gelatin having a strong tendency to fog there is added a solution of 10 milligrams of guanine in a mixture of 10 cc. of water and 2 cc. of

5

$\frac{n}{10}$  NaOH

on 1 kilo of dry gelatin, before the gelatin is made up into an emulsion.

Example 2.—To a photographic silver halide emulsion prepared from a gelatin having a high tendency to fog there is added, before the emulsion is cast, a solution of 10 milligrams of a mixture of equal parts of guanine and adenine in 10 cc. of water and 2 cc. of

10

15

$\frac{n}{10}$  NaOH

on 1 kilo of dry gelatin.

20

What we claim is:

1. A photographic silver halide gelatin emulsion containing amino purines in an amount of about 10 milligrams per kilo of dry gelatin.

2. A photographic silver halide gelatin emulsion containing guanine in an amount of about 10 milligrams per kilo of dry gelatin.

3. A photographic silver halide gelatin containing a mixture of guanine and adenine in an amount of about 10 milligrams per kilo of dry gelatin.

25

30

E. J. BIRR.  
HANS FRICKE.  
GUSTAV WILMANNS.